

## UNITED STATES PATENT OFFICE.

LEWIS W. MALLASEE, OF PITTSBURGH, PENNSYLVANIA, ASSIGNOR TO WILLIAM H. MALLASEE, OF PITTSBURGH, PENNSYLVANIA.

## FERROUS ALLOY.

No Drawing.

Application filed September 22, 1927. Serial No. 221,402.

This invention relates to a ferrous alloy, and to the method of making the same.

An object of the invention is to provide a steel of increased toughness, that is of increased tensile strength, without detracting from the inherent hardness of the steel and with an increase in the ability of the steel to take a high temper.

Another object of the invention is to provide an alloy which is dense and homogeneous in its structure, and which is stainless and resistant to corrosion.

Another object of the invention is to provide an alloy, having these qualities, in which the alloying materials are relatively inexpensive, thus permitting their use in steel of various grades to be used for various purposes.

When the steel is made by the crucible process, the alloy is introduced into the pot at the end of the melt, and approximately ten minutes before pouring. When it is made by the open hearth process, it is preferably introduced after the blast has been discontinued and before the metal is poured from the converter, or may be placed in the ladle. The reason for this general time element is to secure a thorough dissemination of the alloy through the molten metal, while avoiding the introduction of the alloy so early in the process of making the steel as to give an unnecessary opportunity for the volatilization and consequent loss of the alloying material.

The alloy used is tin, which is associated with a suitable material, such as aluminum, capable of fluxing in the molten ferrous metal and preventing the volatilization of the tin therefrom. The tin is introduced in a quantity no less than one and one-half ounces of tin for each hundred pounds of the ferrous metal. It has been found that tin in a materially less quantity fails to contribute the desired qualities to the steel in such degree as to render its use of material advantage. The greatest efficiency is obtained by adding the tin in the quantity of two and one-half ounces of tin in each hundred pounds of the ferrous metal. It has been found that when tin in excess of two and one-half ounces for each hundred pounds of ferrous metal is added, the additional advantageous effect is not in proportion to the increased quantity of the alloy. It should be understood that for certain purposes tin

in excess of two and one-half ounces per hundred pounds of ferrous metal may be added. The effect of the tin is obtained irrespective of the carbon content of the steel. With low carbon steel, such as sixty carbon steel, however, the effect is more marked, because a proportionally greater improvement in the quality of the steel is obtained. This is of great importance in that it permits an improvement in the quality of steel for railway rails, structural use, and the like, by the employment of an alloying material of relatively low cost.

With the tin aluminum is added in a quantity at least equal to that of the tin. Both substances should be in the elemental, or metallic state, and desirably in divided form such as the form of shot.

The quantity of aluminum, as given, is in excess of that employed when the function of the aluminum is merely to remove gases from the melt and prevent their occlusion in the ferrous metal. The aluminum oxidizes to form a thick coating over the molten metal in the receptacle, thereby apparently preventing the escape of volatilized tin and enforcing its thorough dissemination through the body of ferrous metal. It is not at present known if any portion of the aluminum remains in the metallic mass, and whether or no it has any more specific effect in causing the inclusion of the tin therein.

The resulting ferrous alloy possesses highly advantageous qualities. It possesses an increased tensile strength, without a diminution of its inherent hardness and with increased capacity to receive a high temper. It has an unusual resistance to corrosion, and has a surface which does not stain upon contact with mild acids and other substances which usually produce such effect. Apparently a body of the metallic alloy is unusually dense and homogeneous, as it possesses unusual resonance and clearness of tone when struck.

What I claim is:

1. The method of making a ferrous alloy which consists in adding tin and aluminum to the ferrous metal while it is in a molten condition and at a pouring temperature.
2. The method of making a ferrous alloy which consists in adding tin and aluminum to the ferrous metal while it is in a molten condition and at a pouring temperature, the ingredients being added in a quantity no less

than one and one-half ounces of each for each hundred pounds of the ferrous metal.

3. The method of making a ferrous alloy which consists in adding tin and aluminum to the ferrous metal while it is in a molten condition and at a pouring temperature, the ingredients being added in a quantity of approximately two and one-half ounces of each for each hundred pounds of the ferrous metal.

4. The method of making a ferrous alloy which consists in adding tin and aluminum to the ferrous metal while it is in a molten condition and at a pouring temperature, the tin being added in a quantity no less than 15 one and one-half ounces of tin for each hundred pounds of the ferrous metal.

In witness whereof, I hereunto set my hand.

LEWIS W. MALLASEE.